

Nov. 18, 1941.

H. J. DAILEY

2,263,164

ANODE

Filed Feb. 25, 1941

*Fig. 1.*



*Fig. 2.*



*Fig. 3.*



INVENTOR

H. J. DAILEY

BY

*J. W. Greenhow*  
ATTORNEY

## UNITED STATES PATENT OFFICE

2,263,164

## ANODE

Hampton J. Dailey, Bloomfield, N. J., assignor to  
 Westinghouse Electric & Manufacturing Company, East Pittsburgh, Pa., a corporation of Pennsylvania

Application February 25, 1941, Serial No. 380,417

7 Claims. (Cl. 250—27.5)

My invention relates to discharge devices, and especially to the anode structure therein.

An object of the invention is to provide an anode with good gas-absorbing qualities.

A still further object of the invention is to provide a gas-absorbing anode that is easily fabricated to close dimensions and inexpensive.

Other objects and advantages of the invention will be apparent from the following description and drawing in which:

Fig. 1 is an elevational view of a typical discharge device embodying my invention.

Fig. 2 is a cross-sectional view through the anode of Fig. 1 illustrating a preferred embodiment of my invention.

Fig. 3 is an enlarged cross-sectional view of a small portion of the electrode base and coating.

One of the problems in industrial tubes has been the liberation of gases during operation which change the operating characteristics of the tube. Heretofore tantalum has been utilized in view of its gas-absorbing qualities. Tantalum, however, is very expensive.

It is an object of my invention to utilize zirconium because of its good gas-absorbing qualities. The zirconium, however, as heretofore used, scales off easily and has proven unsatisfactory. With my invention, however, I utilize a porous substance, such as graphite, or a roughened metal surface to provide a firm binding base for the zirconium.

In Fig. 1 I have illustrated a typical vacuum tube, such as that adapted for industrial use. This tube comprises a glass casing 10 having a reentrant press 11 at one end through which extend the conductors 12 and 13 to a cathode 14, preferably of the M shape disclosed. This cathode is surrounded by a grid cage 15 supported on standards 16. These standards are supported in turn by certain cross insulators 17, 18, and 19. One of these cross insulators 18 provides means for resiliently supporting the cathode 14 with a spring 20 resiliently supporting a hook 21 for the upper part of the filament. A cross bar 22 in the lower part of the tube supports the grid structure on the lower reentrant press, and from this cross bar 22 is a connection 23 passing through press 11 as a grid lead.

The anode of my invention surrounds the cathode and grid structure. This anode 25 is preferably of the oval cross section disclosed in Fig. 2 and extends axially of the tube the distance of the effective electron-emitting portion of the cathode 14. The anode has its main oval axis

rather elongated in view of the shape of the cathode.

As disclosed in Fig. 2, the inner sides 30 and 31 provide an extensive electron-receiving surface. In order to support the anode I preferably locate eight projecting bosses on the upper and lower portions of both sides of the anode. Two of these bosses 32 and 33 are on the upper portion of the anode in Fig. 1 and symmetrically spaced on each side of the longitudinal axis of the tube. The lower portion of the anode has two similar bosses 34 and 35 aligned with the top bosses. The rear side of the anode has two similar bosses 36 and 37 on the upper portion and two similar bosses, not shown, on the lower portion. These bosses have aligned openings 38 therethrough. Standards 40 are threaded through the aligned openings in each upper and lower pair of bosses and standards 40 are secured in the bottom insulator 19 as disclosed in Fig. 1. The upper ends 41 of these standards are bent over to the reentrant press 42 at the upper end of the tube and secured thereto. A connection 43 extends through the press to the anode exterior connection 44 at the upper end of the tube. The exterior connections for the cathode and grid preferably extend through the lower base 45 of the tube.

In forming the anode I select a porous rough-surfaced material as a base and fabricate it to the desired shape, such as disclosed in Figs. 1 and 2. The material which I have found especially desirable is carbon in the form of graphite. I then mix the zirconium powder with a binder or carrier and preferably utilize a nitrocellulose binder because the volatile constituents are easily baked out and the residue from the binder is essentially carbon. The zirconium powder is preferably of about 325 mesh fineness, and after being mixed with the binder, can be sprayed or painted on the outer surface 46 and inner surface 47 of the carbon base 48 of the anode.

The carbon or roughened metal base can also be immersed in the powder and binder, but this is not as efficient as spraying. The zirconium may also be melted and forced into the pores by an air-blast. The zirconium then cools and solidifies in place. The melting can be performed by having a current passing through a zirconium wire maintained in contact with an electrode and the zirconium sprayed by a hot air blast on the carbon or roughened metal base as the zirconium melts on the electrode. The anode is then assembled in the tube.

I have found that no other baking was necessary than that used in exhausting the tube. One

minute at 1200° C. induction treatment was usually sufficient to eliminate visible ionization in the tube. The binder was baked out and a firmly bonded zirconium layer remained on the carbon anode. The carbon with its surface pores well-filled with the zirconium film, provides a layer which does not easily flake off during operation. The firm bond between the two is illustrated in the enlarged view in Fig. 3.

If a metal base is desired, I roughen the surface, preferably by sand or carborundum blasting, and then fill the artificially made pores with the zirconium layer. The grid 15 may be coated with zirconium to reduce secondary emission.

My invention is also adapted for tubes utilizing mercury vapor as the zirconium absorbs the undesired gases.

My invention has accordingly produced a cheap and easily fabricated anode with good gas-absorbing qualities.

Although I have shown and described a specific embodiment of my invention, I do not desire to be limited thereto as various other modifications of the same may be made without departing from the spirit and scope of the appended claims.

I claim:

1. An electrode for a discharge device comprising a porous base and a coating of zirconium on said porous base with the portion of said coating contiguous to the base embedded in the pores thereof.
2. An electrode for a discharge device comprising a porous carbon base and a coating of

zirconium on said porous carbon base with the portion of said coating contiguous to the base embedded in the pores thereof.

3. The method of treating an electrode to have gas-absorbing properties which comprises selecting a base having large surface pores and filling said pores with zirconium.

4. The method of treating an electrode to have gas-absorbing properties which comprises selecting a base having large surface pores, filling said pores with zirconium powder and a binder and evaporating the binder.

5. A discharge device having a container and cooperating electrodes therein, one of said electrodes comprising a porous material and a coating of zirconium on said porous material bonded to the porous material by portions of the coating entering pores contiguous to said coating.

6. The method of treating an electrode to have gas-absorbing properties which comprises selecting a base having the inherent characteristic of porous rough-surfaced material, and smoothing the exposed surface by both filling the outer pores thereof and coating the surface with zirconium.

7. The method of treating an electrode to have gas-absorbing properties which comprises roughening the exposed surface of a metal base for producing artificial pores, and smoothing the roughened surface by both filling the said artificial pores and coating the surface with zirconium.

HAMPTON J. DAILEY.